

May 1, 1962

TETSURO OSUGI ETAL

3,032,385

PROCESS OF WET SPINNING POLYVINYL ALCOHOL

Filed April 3, 1959



INVENTORS  
TETSURO  
KENICHI  
BY TAKANI  
OSUGI  
TANABE  
MOCHIZUKI

*William C. Long*  
ATTORNEY

1

3,032,385  
PROCESS OF WET SPINNING POLYVINYL  
ALCOHOL

Tetsuro Osugi, Kenichi Tanabe, and Takani Mochizuki, Kurashiki City, Japan, assignors of one-fourth to Air Reduction Company, Incorporated, New York, N.Y., a corporation of New York, and three-fourths to Kurashiki Rayon Co., Ltd., Okayama Prefecture, Japan, a corporation of Japan

Filed Apr. 3, 1959, Ser. No. 803,851

Claims priority, application Japan Apr. 12, 1958  
6 Claims. (Cl. 18—54)

This invention relates to the manufacture of synthetic filaments. More particularly, this invention pertains to a novel method for producing synthetic fibers of the polyvinyl alcohol type which have improved mechanical properties, and to a novel apparatus for carrying out the process.

Synthetic filaments of the polyvinyl alcohol type are usually formed by extruding a solution of the synthetic filament-forming material through small holes in a spinning jet into a liquid wherein the fine streams of extruded solution coagulate or solidify to form filaments. A widely used spinning method for spinning polyvinyl alcohol filaments is described, for example, in U.S. Patent 2,642,333, and copending application Serial No. 336,166 of Tomonari et al., filed February 10, 1953, and now Patent No. 2,988,802. In these processes the polyvinyl alcohol solution is extruded into an up-flowing column of a coagulating liquid having a higher specific gravity than the polyvinyl alcohol solution, thus imparting to the coagulating column and polyvinyl alcohol solution a parallel upward direction of flow without turbulence. The parallel flow is maintained until the polyvinyl alcohol coagulates into filaments. The diameter of the column is subsequently reduced, thereby increasing the rate of flow, and stretching the coagulated filaments by the combined effect of the increased rate of flow and the uplift of the filaments in the coagulating liquid.

Increasing the temperature of the coagulating bath is known to substantially improve the mechanical properties of the fibers produced. Unfortunately, however, when higher temperatures are used in the coagulating bath, adhesion of the filaments occurs when the fibers are taken out of the bath and wound up. For example, when the spinning was carried out at 80° C. in a coagulating bath containing less than 25% by weight of Glauber's salt, less than 35% by weight of ammonium sulfate, and less than 18% by weight of sodium carbonate, the fibers adhered with each other after being taken out of the coagulating bath. The fiber bundles, after being roller-stretched 300% by the usual method and dried by heating, were seen to adhere to each other by inspection of a cross section under the microscope. Moreover, the tensile strengths of the resulting fibers decreased as the bath temperature increased. The tensile strengths of the fibers produced by using bath temperatures of 25° C., 50° C. and 80° C. were found to be 4.3, 3.6 and 2.3 grams per denier respectively. Similar results were obtained when the spinning was carried out using a coagulating bath containing 20% by weight of Glauber's salt at 60° C. Therefore, spinning methods which merely use a higher temperature for the coagulating salt bath are unsatisfactory, in that any advantages which are obtained in improved mechanical properties of the fibers, are lost due to the later adhesion of the fibers when they leave the coagulating bath under the high temperature conditions. Moreover the mechanical advantages may later be lost in the course of stretching the fibers.

A principal object of this invention is to provide a method for producing polyvinyl alcohol filaments hav-

2

ing the improved physical properties which are brought about by the use of higher temperatures in the coagulating bath, without adhesion of the fibers with one another after leaving the coagulating bath, and without loss of valuable mechanical properties on stretching.

Another object of the invention is to provide a polyvinyl alcohol fiber having improved physical characteristics and being suitable as a synthetic fiber for the manufacture of textiles.

Other objects and advantages of the invention will be apparent from a consideration of the specification and claims.

The attached drawing illustrates a spinning apparatus useful in the invention.

According to the present invention, a solution of the filament-forming material is extruded in the form of fine streams into a coagulating liquid having a temperature above 72° C. After coagulation of the fine streams of spinning solution at a temperature above 72° C. the temperature of the bath is lowered to below 58° C. before exit therefrom of the coagulated filaments in order to prevent later adhesion of the filaments and possible loss of valuable mechanical properties on stretching.

In a preferred practice of the invention the initial spinning conditions are regulated in the manner described in U.S. Patent 2,642,333 and co-pending application Serial No. 336,166 of Tomonari et al., filed February 10, 1953. In accordance with the present invention, the upflowing column of coagulating liquid is maintained at a temperature above 72° C. and the spinning solution is coagulated therein. Prior to departure of the coagulated filaments from the coagulation bath, the bath temperature is adjusted to below 58° C. to cool the filaments sufficiently such that the filaments do not adhere to each other with resulting deterioration upon leaving the coagulating bath. The time of contact of the filaments with the coagulating bath portions at different temperatures will depend upon the bath temperatures, the speed of flow of the coagulating bath, the filament speed, the immersion length, and the like.

Improved fibers are obtained when the coagulating bath temperature is maintained above 72° C. through most of the immersion length. Temperatures up to 90° C. have been found to give excellent results. The temperature at which the filaments leave the bath is preferably kept below 58° C. Temperatures as low as 40° C. give good results.

Various means may be employed to provide that the fibers contact coagulating solution of lower temperature when leaving the bath. For example, means whereby the latter part of the coagulating solution is cooled by indirect heat exchange can be employed. Methods in which a part of the coagulating solution of high temperature is removed from the bath during the course of coagulation, as well as the method of feeding or injecting some coagulating solution at a lower temperature can be used. A suitable apparatus for feeding in coagulating solution at a lower temperature is shown in the attached drawing.

Referring now to the attached drawing, the spinning solution is extruded vertically upward through the multi-hole spinneret 1 into contact with the coagulating bath in the lower zone A of the spinning apparatus. The coagulating bath is introduced into the spinning apparatus upwardly through ports 2. In the lower zone of the spinning apparatus the coagulating bath gradually increases in velocity. The extruded fine streams of spinning solution are carried upwardly and coagulated and gently stretched. In the middle zone B of the spinning apparatus the filaments are further coagulated and stretched. Enlarged zone C is provided near the top of the spinning column. Lines 3 are provided for removing

a part of the coagulating bath. Additional coagulating bath which is at a lower temperature is introduced into zone C through lines 4. The coagulating bath overflows at 5 and may be collected and reused by means not shown. Illustrative temperatures of the coagulating bath introduced through lines 2 and 4 are shown on the drawing as well as illustrative temperatures in the different zones of the spinning apparatus. Also shown are illustrative lengths of the various sections of the spinning apparatus.

Salts to be used as the coagulating solution should have the ability to coagulate polyvinyl alcohol aqueous solution at a temperature higher than 72° C. Salts such as, for example, Glauber's salt, ammonium sulfate, potassium sulfate, zinc sulfate, magnesium sulfate, aluminum sulfate and sodium chloride may be used. The coagulating solution which flows in at a lower temperature when the fibers leave the bath is preferably the same kind and the same concentration as the initial coagulating bath, but salts of a different kind and concentration may also be employed. Solutions of higher coagulating power and concentration bring about more favorable results.

The invention will be described in greater detail in conjunction with the following examples, which are typical, but the invention is not limited to the details thereof.

#### Example 1

Polyvinyl alcohol having a degree of polymerization of about 1700 was dissolved in water to form a spinning solution containing 15% by weight of polyvinyl alcohol. This solution was spun at 78° C. to form filaments in the vertical spinning machine illustrated in the accompanying drawing. The polyvinyl alcohol solution was extruded through a spinneret jet having 600 holes, each of 0.08 mm. diameter. The coagulating bath contained 30% by weight sodium sulfate and had an initial speed of 4 m./min. and an exit speed of 10 m./min.

The spun filaments travelled upwardly through the column where a sodium sulfate salt solution at 30° C. was supplied to the upper bath zone as illustrated so that the resulting temperature in this part was 45° C. The filaments were then taken out of this bath.

A part of the filaments (the first series) was wound up and then air-dried at 230° C. The filaments were then heat-stretched 300% within 10 seconds, and afterwards heat-treated at 235° C. for 30 seconds under constant length.

A part of the filaments (the second series) was roller-stretched 300%, dried by heating, and heat-treated at 235° C. for 30 seconds at constant length.

To illustrate the invention, the mechanical properties of the fibers so obtained were compared with fibers coagulated at 28° C., 50° C. and 60° C. bath temperatures in which there was no cooling when the filaments left the bath. These latter fibers were stretched and heat-treated in the same manner as the first series above.

|                                       | The First Series |     |           | The Second Series |
|---------------------------------------|------------------|-----|-----------|-------------------|
|                                       | Comparative Runs |     | Invention | Invention         |
| Bath Temp., ° C.....                  | 28               | 50  | 60        | 78-45             |
| Denier.....                           | 2.7              | 2.6 | 2.5       | 2.6               |
| Strength after dried (g./d.).....     | 4.1              | 4.2 | 4.3       | 5.1               |
| Elongation after dried (percent)..... | 28               | 40  | 42        | 37                |
| Wet Strength (g./d.).....             | 3.3              | 3.4 | 3.4       | 4.1               |
| Dry knot strength (g./d.).....        | 3.5              | 3.8 | 3.9       | 4.4               |
|                                       |                  |     |           | 4.0               |

The data given in the above table for the common strength, knot strength, and elongation of the fibers obtained by spinning in high temperature bath, followed by lowering the exit temperature according to the present invention show that superior filaments are produced. Moreover, when roller-stretching was later applied no deterioration of the quality of the fiber occurred. The fibers which were wound up after being taken out of

the bath, and subsequently air dried, heated and dried, and subjected to roller-stretching, showed no adhesion with each other, by inspection of a cross section with a microscope.

5 The fibers made according to this invention also have improved transparency. When the fibers are chemically acetylated by reaction with formaldehyde they will be dyed to a deeper color per unit equivalent of dyestuff used.

10 The reason for the better physical properties of the fibers obtained by reducing the exit temperature according to this invention is not certain but the following two experiments possibly give some explanation.

(1) Microscopic examination of the fibers produced

15 at bath temperatures of 28° C. and 50° C. produced bright spots on the outer periphery of the fiber and this tendency was greater at 28° C. The fibers produced at bath temperatures of 78° C. showed only dark spots. No bright spots could be observed at all. This showed that

20 a certain change in the arrangement of the molecules occurs on coagulation at different temperatures. A higher arrangement occurs at a lower temperature, but such arrangements do not occur at all at a higher temperature.

(2) Films of an aqueous solution of polyvinyl alcohol

25 on a glass plate were coagulated by using aqueous solutions of 30% Glauber's salt at 25° C., 50° C. and 75° C. respectively. The films were irradiated with X-ray parallel to the surface thereof. The reflection intensity of the X-ray at about 20° of  $\alpha\theta$  on the infra-red ray in the

30 direction normal to the surface of the film was examined by Geiger counter. The intensity increased with increasing coagulating bath temperature. The intensity was -0.84 for the 28° C. film and -0.97 for the 75° C. film. These results show that the plane of the polyvinyl

35 alcohol molecular chains is parallel to the surface of the film at a low temperature coagulations and that such arrangements are few at a high temperature. Therefore, it can be assumed that at high coagulation temperature segments or molecules of polyvinyl alcohol are comparatively in a free state without restriction. Accordingly,

40 with the fibers coagulated at a higher temperature the polyvinyl alcohol segments are in a free state, and more favorable properties are imparted to these fibers when they are later stretched.

#### Example 2

Polyvinyl alcohol having a degree of polymerization of about 2700 was dissolved in water to form a spinning solution containing 14% by weight of polyvinyl alcohol. The polyvinyl alcohol solution was extruded through

50 spinnerets into an aqueous solution containing by weight 30% sodium sulfate with a coagulating bath length of 2 m. The temperature near the spinneret was 90° C., and the exit temperature was 45° C., with substantially a linear temperature gradient in-between. After leaving

55 the bath at a speed of 30 m./min., the fibers were given continuous roller-stretch treatment of 200%. The fibers were then dried and subjected to heat treatment at constant length at 235° C. for one minute. Comparison of these fibers with those obtained under the same conditions except that the coagulating temperature was kept at a constant 45° C. temperature is shown below:

|                                           |          |      |
|-------------------------------------------|----------|------|
| Temperature of coagulating bath, ° C..... | 90 to 45 | 45   |
| Strength, g./d.....                       | 2.23     | 1.75 |
| Elongation, percent.....                  | 34       | 32   |

#### Example 3

Polyvinyl alcohol having a degree of polymerization of about 1600 was dissolved in water to form a spinning solution containing 25% by weight of polyvinyl alcohol. The polyvinyl alcohol solution was extruded through a spinneret into an aqueous solution containing 37% by weight of zinc sulfate. The length of the coagulating bath was 50 cm. and its temperature 80° C. Saturated

aqueous solution of sodium sulfate at 35° C. was poured therein at a distance of 10 cm. from the exit of the coagulating bath to give an exit bath temperature of 48° C. The bath exit speed was 5 m./min. The fiber was then roller-stretched continuously 300%, dried by an infra-red ray, and stretched further 100% for 10 seconds at 240° C. The fiber was then contracted 15% in 10 seconds at 240° C. and formalized at 50° C. for one hour in a solution containing 5% formaldehyde, 15% sulfuric acid and 5% sodium sulfate.

The fibers obtained by the above process were compared with fibers prepared similarly wherein the zinc sulfate coagulating bath was maintained at 45° C. temperature and Glauber's salt solution at 45° C. was added near the bath exit.

|                                           |          |      |
|-------------------------------------------|----------|------|
| Temperature of coagulating bath, ° C..... | 80 to 48 | 45   |
| Strength (g./d.).....                     | 6.54     | 5.26 |
| Elongation (percent).....                 | 18       | 12   |

#### Example 4

Polyvinyl alcohol having a degree of polymerization of about 980 was dissolved in water to form a spinning solution containing 19% by weight of polyvinyl alcohol. The polyvinyl alcohol solution was extruded through spinnerets into an aqueous solution containing 42% by weight of ammonium sulfate. The length of the coagulating bath was 1.5 m. and its temperature 75° C. A part of the coagulating bath flowed out at a distance of 50 cm. from the exit of the bath, and a coagulating solution at 40° C. containing 42% of ammonium sulfate by weight was poured therein. The temperature of the bath when the fiber left the bath was thus brought to 40° C.

The fiber prepared as above was compared with a fiber spun in a bath containing 42% ammonium sulfate by weight at a constant temperature of 40° C. Both of the fibers were stretched as long as possible in 35% ammonium sulfate solution at 90° C. After drying, their strengths and elongations were measured.

|                                           |                 |     |
|-------------------------------------------|-----------------|-----|
| Temperature of coagulating bath, ° C..... | 75 to 40        | 40  |
| Maximum elongation (percent).....         | 42 <sup>1</sup> | 350 |
| Strength (g./d.).....                     | 3.8             | 2.6 |

#### Example 5

Polyvinyl alcohol having a degree of polymerization of about 1700 was dissolved in water to form a spinning solution containing 15% by weight of polyvinyl alcohol. The polyvinyl alcohol solution was extruded through a spinneret into an aqueous solution containing 30% by weight of sodium sulfate. The length of the coagulating bath was 1.5 m. and the temperature was 78° C. An aqueous solution containing 30% by weight of Glauber's salt at a temperature of 35° C. was poured therein. The bath temperature when the fiber left the bath was 53° C. Spinning was effected at a bath exit speed of 40 m./min. The fiber was roller-stretched continuously 150%, dried by an infra-red ray, and then wound up. The fibers thus obtained were stretched as long as possible for 10 seconds at 245° C., and then formalized at 50° C. for one hour in a solution containing 5% formaldehyde, 15% sulfuric acid and 10% sodium sulfate.

The fibers prepared as described above were compared to fibers treated similarly to the above process in a coagulating bath at a constant temperature at 45° C. and at a constant temperature of 78° C.

|                                           |          |     |     |
|-------------------------------------------|----------|-----|-----|
| Temperature of coagulating bath, ° C..... | 78 to 53 | 45  | 78  |
| Dry strength (g./d.).....                 | 8.6      | 6.3 | 5.8 |
| Elongation (percent).....                 | 8        | 9   | 12  |

The fibers prepared by the invention had homogeneous cross section and good dyeing characteristics.

#### Example 6

Polyvinyl alcohol solution having a degree of polymerization of about 500, which was acetalized to an acetalization degree of 30 mole percent using  $\beta$ -cyclohexylaminobutyraldehyde, was mixed with polyvinyl alcohol having a degree of polymerization of about 2200 to have an average aminoacetalization degree in the polymer of 1%. This mixture was dissolved in water to form an aqueous spinning solution having a polymer concentration of 13%. The polyvinyl alcohol solution was extruded through a spinneret into a coagulating bath of saturated aqueous solution of sodium sulfate, the bath having a temperature of 75° C. The immersion length was 2 m. and the exit speed 10 m./min. A saturated aqueous solution of sodium sulfate at a temperature of 35° C. was poured in at a distance of 1 m. from the exit, making the temperature of the bath 42° C. when the fiber left the bath.

The fibers thus obtained were stretched 300% for 1 minute in nitrogen at 220° C. and further heat-treated for 1 minute at constant length in water vapor at 225° C. under one atmosphere pressure. The fibers were then acetalized in an aqueous solution containing 1% benzaldehyde, 5% sulfuric acid and 10% methanol at 60° C. for one hour.

The fibers obtained by the above process were compared with fibers treated similarly except that the coagulating bath temperature was 42° C. throughout.

|                                           |          |      |
|-------------------------------------------|----------|------|
| Temperature of coagulating bath, ° C..... | 75 to 42 | 42   |
| Strength (g./d.).....                     | 3.82     | 2.65 |
| Elongation (percent).....                 | 25       | 24   |

We claim:

1. The method of preparing improved polyvinyl alcohol fibers which comprises forming an aqueous polyvinyl alcohol spinning solution, extruding the said spinning solution in the form of fine streams into a warm coagulating salt solution bath having a temperature above 72° C., coagulating the said fine streams in said warm coagulating solution to form filaments, contacting the said filaments with a cool coagulating solution bath having a temperature lower than 58° C. substantially immediately after contact with said warm solution for a time sufficient to prevent subsequent adhesion of the filaments to each other upon leaving the cool coagulating solution bath, and withdrawing the filaments from the cool coagulating solution bath.

2. In the process for wet-spinning polyvinyl alcohol fibers by extruding fine streams of polyvinyl alcohol solution into an up-flowing column of a coagulating liquid having a higher specific gravity than said polyvinyl alcohol solution, imparting to said coagulating column and said fine streams of polyvinyl alcohol a parallel upward direction of flow without turbulence, maintaining said unturbulent parallel flow until the polyvinyl alcohol coagulates to filaments, subsequently reducing the diameter of said column, thereby increasing the rate of flow thereof, and stretching said coagulated filaments by said increased rate of flow and the uplift of the filaments in the specifically heavier column of the coagulating liquid, the improvement which comprises maintaining the up-flowing column of coagulating liquid at a temperature above 72° C. until the fine streams of polyvinyl alcohol coagulate to form filaments and subsequently reducing the temperature of the coagulating liquid in contact with the filaments to below 58° C. to form a cool coagulating solution bath, the contact with said cool solution being for a time sufficient to prevent adhesion of the filaments to each other upon leaving the cool coagulating solution bath.

3. A method of preparing improved polyvinyl alcohol fibers which comprises the steps of forming an aqueous polyvinyl alcohol spinning solution, extruding said spinning solution in the form of fine streams upwardly into a warm coagulating salt solution bath having a tempera-

ture above 72° C., coagulating said fine streams in said coagulating solution to form filaments, contacting said filaments with a cool coagulating solution bath having a temperature lower than 58° C. substantially immediately after contact with said warm solution for a time sufficient to prevent subsequent adhesion of the filaments to each other upon leaving the cool coagulating solution bath, and withdrawing the filaments from said cool coagulating solution bath.

4. A method of preparing improved polyvinyl alcohol fibers which comprises the steps of forming an aqueous polyvinyl alcohol spinning solution, extruding said spinning solution in the form of fine streams into a warm coagulating salt solution bath having a temperature of 72° to 90° C., coagulating said fine streams in said coagulating solution at said temperature to form filaments, contacting said filaments with a cool coagulating solution bath having a temperature of 40° to 58° C. substantially immediately after contact with said warm solution for a time sufficient to prevent subsequent adhesion of the filaments to each other upon leaving the cool coagulating solution bath, and withdrawing the filaments from said cool coagulating solution bath.

5. A method of preparing improved polyvinyl alcohol fibers which comprises the steps of forming an aqueous polyvinyl alcohol spinning solution, extruding said spinning solution in the form of fine streams upwardly into a warm coagulating salt solution bath having a temperature of 72° to 90° C., coagulating said fine streams in said coagulating solution at said temperature to form filaments, contacting said filaments with a cool coagulating solution bath having a temperature of 40° to 58° C. substantially immediately after contact with said warm solution for a time sufficient to prevent subsequent adhesion of the filaments to each other upon leaving the cool coagulating

8  
solution bath, and withdrawing the filaments from said cool coagulating solution bath.

6. In the process for wet-spinning polyvinyl alcohol fibers by extruding fine streams of polyvinyl alcohol solution into an up-flowing column of a coagulating liquid having a higher specific gravity than said polyvinyl alcohol solution, imparting to said coagulating column and said fine streams of polyvinyl alcohol a parallel upward direction of flow without turbulence, maintaining said turbulent parallel flow until the polyvinyl alcohol coagulates to filaments, subsequently reducing the diameter of said column, thereby increasing the rate of flow thereof, and stretching said coagulated filaments by said increased rate of flow and the uplift of the filaments in the specifically heavier column of the coagulating liquid, the improvement which comprises maintaining the up-flowing column of coagulating liquid at a temperature of 72° to 90° C. until the fine streams of polyvinyl alcohol coagulate to form filaments, and subsequently reducing the temperature of the coagulating liquid in contact with the filaments to 40° to 58° C. to form a cool coagulating solution bath for a time sufficient to prevent adhesion of the filaments to each other upon leaving the cool coagulating solution bath.

References Cited in the file of this patent

UNITED STATES PATENTS

|           |                 |                |
|-----------|-----------------|----------------|
| 1,906,042 | Barthelemy      | Apr. 25, 1933  |
| 2,467,541 | Taylor          | Apr. 19, 1949  |
| 2,536,094 | McDermott       | Jan. 2, 1951   |
| 2,610,359 | Hatchard et al. | Sept. 16, 1952 |
| 2,636,217 | Hammond         | Apr. 8, 1953   |

FOREIGN PATENTS

|         |        |              |
|---------|--------|--------------|
| 561,291 | Canada | Aug. 5, 1958 |
|---------|--------|--------------|